

# UNITED STATES PATENT OFFICE.

JOHN J. VARN BUHLER, OF DETROIT, MICHIGAN.

## RUST-REMOVING COMPOUND.

No Drawing.

Application filed December 28, 1921. Serial No. 525,473.

To all whom it may concern:

Be it known that I, JOHN J. VARN BUHLER, a citizen of the United States, residing at Detroit, county of Wayne, State of Michigan, have invented a certain new and useful Improvement in Rust-Removing Compounds, of which the following is a specification.

My invention relates to a metal cleaning compound intended particularly for use in cleaning surfaces of metal parts which are subsequently to be painted or enameled. In a companion application filed December 28, 1921, Serial No. 525,472, I have described and claimed broadly a metal cleaning compound composed essentially of a rust preventing liquid, an acid such as hydrochloric acid which will not unite with the rust-preventing liquid, and alcohol. The present invention relates to a more specific form of the compound therein described, the present compound being intended particularly for use as a second treatment for metallic parts which have been treated with the compound containing linseed oil, such as is described in my hereinbefore mentioned application, or with some other rust removing compound, or for use where the articles are not deeply rusted or heavily coated with foreign substances.

The compound embodying my present invention comprises in its preferred form equal parts of hydrochloric acid and glycerine combined with two parts of alcohol. In practice, I employ wood alcohol and apportion the ingredients by volume. I also add, if desired for the particular purpose for which the compound is to be used, ten percent of distilled water. Thus in practice, I use 32 ounces of hydrochloric acid, 32 ounces of glycerine and 64 ounces of wood alcohol. To these ingredients when thoroughly mixed, I add a tenth of a gallon of distilled water if a thinner or weaker compound is preferred.

What I claim is:

1. The metal cleaning compound containing glycerine, hydrochloric acid, and alcohol.
2. The metal cleaning compound comprising about 32 ounces of glycerine, 32 ounces of hydrochloric acid and 64 ounces of alcohol and one-tenth of a gallon of distilled water.
3. The metal cleaning compound containing one part each of glycerine and hydrochloric acid and two parts of alcohol.

In testimony whereof I affix my signature.

JOHN J. VARN BUHLER.